

(No Model.)

3 Sheets—Sheet 1.

J. C. BULL.

APPARATUS FOR SMELTING AND REFINING COPPER.

No. 520,631.

Patented May 29, 1894.



Witnesses:

H. G. Dieterich  
B. W. Sommers

Inventor:  
Johannes C. Bull.

by Henry M. Atty.

(No Model.)

3 Sheets—Sheet 2.

J. C. BULL.

APPARATUS FOR SMELTING AND REFINING COPPER.

No. 520,631.

Patented May 29, 1894.



Witnesses:

H. G. Dieterich  
B. H. Sommers

Inventor:

Johannes C. Bull.  
or Henry W.  
Atty:

(No Model.)

3 Sheets—Sheet 3.

J. C. BULL.

APPARATUS FOR SMELTING AND REFINING COPPER.

No. 520,631.

Patented May 29, 1894.



*Witnesses:*  
H. G. Dieterich  
P. H. Sommers

*Inventor:*  
Johannes C. Bull.  
by Henry M.  
*Atty:*

# UNITED STATES PATENT OFFICE.

JOHANNES C. BULL, OF ERITH, ENGLAND.

## APPARATUS FOR SMELTING AND REFINING COPPER.

SPECIFICATION forming part of Letters Patent No. 520,631, dated May 29, 1894.

Application filed May 12, 1891. Serial No. 392,498. (No model.)

*To all whom it may concern:*

Be it known that I, JOHANNES CATHARINUS BULL, engineer, a subject of the King of Sweden and Norway, residing at Erith, in the county of Kent, England, have invented certain new and useful Improvements in Apparatus for Smelting and Refining Copper, of which the following is a specification, reference being had to the accompanying drawings.

- 10 My invention relates to improvements in apparatus for the smelting and refining of copper obtained from ores, mattes or other cupriferous materials by oxidation which is attained by the introduction of nitrates or 15 other similar substances into the copper below the surface thereof while the metal is in a melting or molten state in measured and controllable quantities and at a controllable speed.
- 20 In order that my invention may be more easily understood I will describe the same with reference to the accompanying drawings, of which—

Figure 1 is a sectional elevation of a converter somewhat after the style of a Bessemer converter and suitable for refining small quantities of copper say three or four hundred-weight at a time. Fig. 2 is a similar view of a converter adapted for working on a somewhat larger scale. Fig. 3 is a sectional elevation of apparatus which I prefer to use in working my invention commercially. Fig. 4 is a sectional plan view on line X Y Fig. 3, and Fig. 5 is a side elevation partly in section on line Z Z Fig. 3.

The same letters of reference refer to similar or equivalent parts in all the drawings.

I prefer to use as shown on the drawings a furnace or converter A of the "Bessemer converter" type provided with trunnions d to allow of inversion.

Referring more particularly to Fig. 1, the bottom part a' can be bolted or otherwise fixed onto the converter A. I prefer to make the lining A' of the converter and the bottom part of "ganister" or other suitable fireproof material such as a mixture of sand and clay. In the bottom part a' of the converter A is firmly embedded an open vessel b with a conical or 50 other suitably shaped upper part or top c, both made of fire clay or other refractory material. The top c has a number of holes c',

say from ten to fifteen, of a diameter of from one-fourth to three-eighths of an inch. The conical top c of the vessel b has the same taper as a metal fin a formed on the bottom of the converter and the lining A' thereof after the point when the said fin a ceases, so that the top c is kept in place by the fin and the lining when the bottom part a' is fixed in its place.

In using this form of converter or furnace I proceed as follows:—Into the vessel b I introduce oxidizing agents such as nitrate or chlorate of soda or potash, the cover c is then put on and the bottom part a' is fixed in its place at the bottom by means of bolts as shown or in any other convenient manner. The weight of the charge of nitrate of soda corresponds to about five per cent. of that of the copper intended to be refined and in these proportions good results have been obtained. It should however be noted that the amount of oxygen produced by different oxidizing agents varies and the proportions have to be varied to suit different cases and that whenever the expression "nitrate" is used herein it should be understood that any suitable oxidizing agent is intended. The impure copper is melted with a suitable slag for the scoriaction of ferrous and other oxides while in the converter and is then poured into the said converter A whereupon a portion of it will sink through holes c' into the vessel b, and by the intense heat, decompose part of the "nitrate" and cause a strong current of oxidizing gases or matter to pass up and through the molten copper which gases for a time exert sufficient pressure to prevent further quantities of the copper from entering the vessel b. After a while however the pressure decreases so that more copper can enter through the lowest holes c', more gases are disengaged and the process is continued until all the "nitrate" or other oxidizing agent in the vessel b is decomposed. The number and size of the holes c' are so arranged that the speed of the decomposition is regulated. During the process the iron is oxidized and scoriaction by the slag which should be rich in silica, the sulphur is oxidized and removed as sulphurous oxide, the arsenic and antimony are oxidized and volatilized at the high temperature developed and the other impurities

are either gasified or scorified by the slag or the lining. When the reaction becomes languid the slag may be removed through the opening closed by a door *f* and the copper, 5 after "poling," tapped through an opening *g* or it may be "poled" outside the converter, or if as shown the converter be invertible the copper may be poured out through its mouth. The bottom part *a'* is then detached and any 10 copper that may remain in the vessel *b* is emptied out, a new charge of oxidizing agent inserted and the process repeated as before described.

When it is required to treat larger quantities the arrangement shown in Fig. 2, Sheet 1, may be conveniently employed. The vessel *b* in this case is replaced by a conical block *c* made of the same material and secured in place by the fins *a* as before described. This block *c* has a horizontal channel *c'* with six or more vertical tapering passages or holes *c'* as shown. The channel *c'* is in communication with a tube *l* which is embedded in the lining of the converter and is 25 provided on the outside of the converter with a stop valve or cock *l'* for opening and shutting off communication with the tube *l* which is lagged or covered with non-conducting material. The tube *l* is carried up above the 30 level of the copper in the converter and communicates with a vessel *b* which is also preferably lagged or coated with non-conducting composition. The vessel *b* is provided with a lamp or other heat producer *n*. The oxidizing agents are introduced into the vessel *b* and melted by heat in a convenient manner and as the impure molten copper is poured into the converter, an air pump *o* is put in motion, the valve *l'* opened and by the air 35 pressure on the surface of the liquid or semi liquid nitrate, jets of the latter are forced into the copper through the holes *c'* at such a rate that about five per cent. of the nitrate compared with the weight of the copper is forced 40 in during a period of from ten to fifteen minutes, providing the copper do not contain more than from five to eight per cent. of impurities. The period is of course extended if the percentage be higher. If the supply of oxidizing 45 agent contained in the vessel *b* be not sufficient for the amount of copper contained in the converter, I may, in order not to interrupt the process provide duplicate parts for the supply of the oxidizing agents or as shown 50 the vessel *b* may be connected to another similar vessel situated at a higher level and connected thereto by a pipe *p* having a cock or valve *p'*, the valve *l'* being closed during the refilling of the vessel to prevent the copper 55 per rising in the tube *l* and opened when sufficient oxidizing agent is obtained ready for the continuation of the supply thereof. Otherwise this form of apparatus works in the same manner as that described with 60 reference to Fig. 1 with this exception that the supply of the nitrate or other oxidizing agent is under better control. If the con-

verter or furnace be of the invertible type the supply pipe *l* is led through the trunnion. The poling must either take place outside the 70 converter or while the latter is laid over so far that the metal cannot enter the channels *c'*. About eight or ten hundred weight is a suitable charge for a furnace of this description. 75

The reason for making the inside bottom of the converter of the approximately coned form shown is that a better distribution of the oxidizing agent is effected while at the same time where required facilities are given 80 for the purest grade of copper to sink below the level of the holes *c'* and the said copper may when desired be easily drawn off by an opening *g* normally closed by a plug. 85

When working on a large scale and particularly when treating "matte," "regulus" or coarse copper with large percentages of impurities I prefer to use a converter constructed on the lines of an ordinary Bessemer converter being however modified to a certain 90 extent to adapt it to the work in question, as shown with reference to Figs. 3 and 4, Sheet 2, and Fig. 5, Sheet 3. In this case I have shown a method of supplying the oxidizing agent in a dry and powdered form by means 95 of a blast. A vessel *b* is filled with the powdered nitrate and closed with a lid *b'* either screwed or sufficiently heavy to prevent its being raised by the pressure of the blast. In the bottom part of the said vessel I mount a 100 wheel *b'* provided with a number of pockets or series of revolving hoppers which wheel is revolved at a controllable speed by any suitable means and thus regulates the amount of powdered nitrate to be discharged from the 105 vessel *b* into the pipe *l* by means of the blast coming from any suitable source by the pipe *o*. The wheel *b'* is fitted to work tightly against the walls of the vessel *b* so that no appreciable amount of blast can pass it into the vessel *b*. I 110 may however also provide a by pass pipe *b'* in order to equalize the pressure above and below the nitrate in the vessel *b*. By regulating the speed of the wheel *b'* which is actuated preferably by worm and worm wheel gear, the 115 amount of powdered nitrate can be accurately controlled. 120

If the copper to be refined contains less than eighty per cent. of metallic copper, say fifty to sixty per cent., the process should proceed as follows:—A suitable charge of say two thousand five hundred to three thousand pounds is melted with some slag rich in silica and poured into the converter in the usual way and the blast is put on, the atmospheric 125 air alone being sufficient to oxidize the impurities at a sufficient rate to keep the metal fluid for some time, but partly to accelerate the reactions and partly to keep the tuyeres *c'* clear and open it is advisable to start the 130 nitrate feeding apparatus at once at a slow rate, the nitrate decomposing at the openings and acting on the impurities of the copper sufficient heat is evolved to make it sure that

the openings do not become choked. To further assist this clearing action I make as shown one or more of the cells or hoppers of the wheel  $b^2$  with a larger capacity than the others thus generating a larger quantity of gases and consequently a great evolution of heat at suitable intervals. During the first fifteen to twenty minutes about one and one-half per cent. of nitrate should be introduced after which the converter is turned over so far that the slag can be removed, the blast stopped or reduced, fresh slag introduced and the blast continued as before for another fifteen or twenty minutes with an injection of two to four per cent. of nitrate, increasing the speed of injection as the amount of impurities and consequently the heat evolved through their combustion diminishes. When the absence of flame and smoke or vapor denotes the end of the process, the metal is poured after poling unless the latter process is carried on outside the converter. With metal having about eighty per cent. or more of metallic copper or when the converter is fixed the process is carried on without interruption to the end. When the "matte" is very poor it may be necessary to pour out the whole of the contents of the converter after the first "blow" in order to give the matte and slag sufficient time to separate, the slag can then be removed and the blast continued.

The oxidizing agent that I prefer to use is Chili saltpeter (nitrate of soda) as being the cheapest and not too violently explosive when subjected to heat but other materials capable of evolving large quantities of oxygen or oxidizing gases or matters or mixtures thereof may be employed. The matters referred to may also be decomposed by heat or otherwise outside of the apparatus and the resulting bodies or gases evolved forced in in any suitable manner.

I have only described and shown apparatus for carrying on the refining process intermittently but it is evident that the latter might be made continuous by passing the refined copper out at the bottom while feeding in the molten unpurified metal.

Having fully described my invention, what I desire to claim and secure by Letters Patent is—

1. An apparatus for refining copper comprising a converter and in combination therewith of a vessel or holder seated centrally in the bottom lining thereof and having a coni-

cal top projecting into the converter above said bottom, the top of said vessel being provided with diverging passages, substantially as and for the purpose set forth.

2. An apparatus for refining copper comprising a converter having the central portion of its bottom constructed in the form of an inwardly projecting cone, said cone being chambered and provided in and about its apex with diverging passages, and a tap hole arranged below the said apex of the cone, substantially as and for the purpose set forth. 60

3. An apparatus for refining copper comprising a converter having a conical seat or bearing formed centrally in its bottom lining in combination with a chambered cone seated in said bearing and projecting beyond the same into the converter, said cone having diverging passages formed in and about its apex, and retaining devices connected with the converter shell having bearing on the sides of the chambered cone, substantially as and for the purpose set forth. 70

4. An apparatus for refining copper comprising a converter, a chambered cone projecting centrally from the converter bottom into the same, said cone provided in and about its apex with diverging passages, a tap hole in the converter wall below the apex of said cone, a receiver for containing an oxidizing agent, a connection between the receiver and the chambered conical bottom of the converter, and a forcing device for forcing the oxidizing agent into and through said chambered bottom, for the purpose set forth. 85

5. An apparatus for refining copper comprising a converter having the central portion of its bottom constructed in the form of an inwardly projecting cone, said cone being chambered and provided in and about its apex with diverging passages, a receiver for holding a dry pulverulent oxidizing agent, a pipe connection between the receiver and the chambered bottom of the converter, a feeding device constructed to feed the oxidizing agent 95 in measured quantities to said pipe connections and a blast pipe in communication with the pipe connections, substantially as and for the purpose set forth. 100

J. C. BULL.

Witnesses:

THOMAS LAKE,  
17 Gracechurch Street, London.

ARTHUR M. FLACK,  
77 Chancery Lane, London.